

## UNITED STATES PATENT OFFICE

2,021,781

ALLOY STEEL AND ARTICLES MADE  
THEREFROM

Walter G. Hildorf, Canton, Ohio, and Albert E. White and Claude L. Clark, Ann Arbor, Mich., assignors to The Timken Roller Bearing Company, Canton, Ohio, a corporation of Ohio, as trustee

No Drawing. Application November 20, 1931,  
Serial No. 576,428

5 Claims. (Cl. 75—1)

Our invention relates to alloy steels and to articles made therefrom which are adapted for use at high temperatures, particularly temperatures above 750° F.

5 The invention has for its principal object an alloy steel and articles made therefrom which will be capable of resisting oxidation at elevated temperatures, that is, above 750° F., which are extremely resistant to shock at such temperatures, which have a high degree of strength, which are easily workable and thus capable of being fabricated into intricate shapes and which will be considerably lower in cost than the austenitic steels or the high chromium steels ordinarily used at such high temperatures.

10 The invention consists principally in an alloy steel containing chromium, tungsten and silicon as its principal alloying ingredients with or without vanadium and having substantially the following composition:

|             | Per cent     |
|-------------|--------------|
| Carbon      | 0.01 to 0.20 |
| Manganese   | 0.20 to 1.0  |
| Silicon     | 0.50 to 1.0  |
| 25 Chromium | 0.75 to 1.50 |
| Tungsten    | 0.50 to 1.50 |
| Vanadium    | 0.01 to 0.50 |

20 with the usual percentages of sulphur and phosphorous.

30 The invention further consists in the alloy steel and articles made therefrom hereinafter described and claimed.

Our alloy steel is suitable for such uses as 35 high temperature steam lines for power plants, superheater tubes, oil still tubes in which sweet crude oil is used and in which corrosion is not a serious factor, for heat exchangers and condensers.

40 It is recognized that chromium-tungsten-silicon steels have heretofore been known but they have been used as tool steels, particularly in the manufacture of tools, such as drills, taps, reamers and chisels, and they have not been regarded as satisfactory for the high temperature uses hereinbefore set forth.

45 The general range of several ingredients of our alloy steel is as follows:

|             | Per cent     |
|-------------|--------------|
| 50 Carbon   | 0.01 to 0.20 |
| Manganese   | 0.20 to 1.0  |
| Silicon     | 0.50 to 1.0  |
| Chromium    | 0.75 to 1.50 |
| Tungsten    | 0.50 to 1.50 |
| 55 Vanadium | 0.01 to 0.50 |

A preferred narrower range of ingredients is as follows:

|           | Per cent     |
|-----------|--------------|
| Carbon    | 0.01 to 0.10 |
| Manganese | 0.20 to 0.60 |
| Silicon   | 0.60 to 1.0  |
| Chromium  | 0.75 to 1.25 |
| Tungsten  | 0.75 to 1.20 |

10 The tungsten content of our steel preferably approximates fairly closely the chromium content thereof, but should not appreciably exceed the chromium content; whereas in prior chromium-tungsten-silicon steels, the tungsten content has been about twice the chromium content. 15 The tungsten content of our steel will ordinarily be somewhat less than the chromium content, so as to avoid the possibility of its appreciably exceeding the chromium content.

20 The preferred narrow range is based upon the results of tests of numerous alloy steels within the broad range of ingredients hereinbefore set forth, including tests of the short time proportional limit at 1000° F. (which is commonly accepted as the best measure of the metal's high 25 temperature creep resistance) load carrying ability, ductility and impact resistance.

Our alloy steel has an actual creep resistance and load carrying ability at 1000° F. far in excess 30 of what was to be expected of chromium-tungsten-silicon alloys; and it has a good combination of strength and ductility at 1000° F.

Said alloy has an excellent combination of 35 strength, ductility and resistance of impact resistance at 75° F. and hence is very well adapted for low temperature use as well as high temperature use. The steel has a good resistance to oxidation at temperatures from 1000° to 1200° F.

40 Following are the results of tests of a typical steel embodying our invention and having the following composition: .025% C, .23% Mn, .46% Si, 1.13% W, 1.20% Cr.

45

## Physical properties at 1000° F.

| Tensile strength lbs. per sq. in. | Proportional limit lbs. per sq. in. | Percent elong. 2" | Percent Red. area | Creep strength 1 percent per 100,000 hrs. |
|-----------------------------------|-------------------------------------|-------------------|-------------------|-------------------------------------------|
| 46,000-50,000                     | 11,000-17,000                       | 26.0-29.5         | 76.5-77.5         | 14,800                                    |

55

## Physical properties at 75° F.

| 5 | Tensile strength lbs. per sq. in. | Proportional limit lbs. per sq. in. | Percent elong. 2" | Percent Red. area | Brinell hardness | Izod impact |
|---|-----------------------------------|-------------------------------------|-------------------|-------------------|------------------|-------------|
|   | 68,200-75,500                     | 35,000-40,000                       | 34.0-37.0         | 72.7-77.5         | 138-153          | 101-104     |

## Percent loss of weight by oxidation in 150 hours

| 10 | 1000° F. | 1100° F. | 1200° F. |
|----|----------|----------|----------|
|    | .35      | .90      | 3.80     |

- 15 The qualities and characteristic features of our alloy steel and articles made therefrom as herein brought out constitute important advantages and satisfy a long existing demand for a low priced steel having such qualities.
- 20 The addition of vanadium in amounts from 0.01% to 0.50% is helpful in improving the properties of the steel at high temperatures.

What I claim is:

- 25 1. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing from about 0.01 to 0.2 per cent of carbon, about 0.75 to 1.5 per cent of chromium, about 0.2 to 1.0 per cent of manganese, about 0.5 to 1.0 per cent of silicon, about 0.5 to 1.5 per cent of tungsten, the tungsten content being less than the content of chrominum, and the remainder of the steel being substantially iron.
- 30 2. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing from about 0.01 to 0.1 per cent of carbon, about 0.75 to 1.25 per cent of chromium, about 0.2 to 0.6 per cent of manganese, about 0.6 to 1.0 per cent of silicon, about 0.75 to 1.2 per cent of tungsten, about 0.01 to 0.5 per cent of vanadium, the tungsten content being less than the content of chromium, and the remainder of the steel being substantially iron.
- 35 3. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing from about 0.01 to 0.1 per cent of carbon, about 0.75 to 1.25 per cent of chromium, about 0.2 to 0.6 per cent of manganese, about 0.6 to 1.0 per cent of silicon, about 0.75 to 1.2 per cent of tungsten, the tungsten content being less than the content of chrominum, and the remainder of the steel being substantially iron.
- 40 4. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing from about 0.01 to 0.1 per cent of carbon, about 0.75 to 1.25 per cent of chromium, about 0.2 to 0.6 per cent of manganese, about 0.6 to 1.0 per cent of silicon, about 0.75 to 1.2 per cent of tungsten, about 0.01 to 0.5 per cent of vanadium, the tungsten content being less than the content of chromium, and the remainder of the steel being substantially iron.
- 45 5. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing from about 0.01 to 0.1 per cent of carbon, about 0.75 to 1.25 per cent of chromium, about 0.2 to 0.6 per cent of manganese, about 0.6 to 1.0 per cent of silicon, about 0.75 to 1.2 per cent of tungsten, the tungsten content being less than the content of chromium, and the remainder of the steel being substantially iron.

the tungsten content being less than the content of chromium, and the remainder of the steel being substantially iron.

3. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing about 0.025 per cent of carbon, about 1.2 per cent of chromium, about 0.23 per cent of manganese, about 0.5 per cent of silicon, about 1.13 per cent of tungsten, and the remainder of the steel being substantially iron.

4. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing from about 0.01 to 0.2 per cent of carbon, about 0.75 to 1.5 per cent of chromium, about 0.2 to 1.0 per cent of manganese, about 0.5 to 1.0 per cent of silicon, about 0.5 to 1.5 per cent of tungsten, about 0.01 to 0.5 per cent of vanadium, the tungsten content being less than the content of chromium, and the remainder of the steel being substantially iron.

5. An article, such as a boiler tube or the like, for use at high temperatures the article being formed from a steel alloy characterized by maintained high creep strength under continuous exposure to operating stress at temperatures in excess of 750° F., by substantial resistance to oxidation at operating temperatures, and by containing from about 0.01 to 0.1 per cent of carbon, about 0.75 to 1.25 per cent of chromium, about 0.2 to 0.6 per cent of manganese, about 0.6 to 1.0 per cent of silicon, about 0.75 to 1.2 per cent of tungsten, about 0.01 to 0.5 per cent of vanadium, the tungsten content being less than the content of chromium, and the remainder of the steel being substantially iron.

WALTER G. HILDORF.  
ALBERT E. WHITE.  
CLAUDE L. CLARK.